

## UNITED STATES PATENT OFFICE

1,980,670

## INHIBITOR FOR NITRIDING PROCESSES

Harold A. Eckman, Oak Park, and Henry W. Maack, Chicago, Ill., assignors to Crane Co., Chicago, Ill., a corporation of Illinois

No Drawing. Application June 20, 1931,  
Serial No. 545,834

5 Claims. (Cl. 134—1)

This invention relates to the surface hardening of ferrous alloys by the nitriding process and more particularly to a means for preventing the hardening of selected parts of articles being treated by the nitriding process to harden surface layers.

In the surface hardening of ferrous alloy articles it is often desirable to prevent certain portions of the articles from being hardened, so as to avoid the resultant brittleness thereof as in the case of screw threaded portions or other parts which may be desired soft for subsequent machining or for other reasons.

We are aware that methods have been used and coatings supplied for selective hardening of steel articles where the hardening of the surface was obtained by a carburizing process but we have found by actual trial of all these known methods and coatings that they are ineffectual in preventing hardening obtained by nitriding processes due to the particular problems and conditions presented by the nitriding processes. We are also aware that it has been proposed to tin portions of the articles not desired to harden. This method however is very costly, requires personal skill and is not satisfactory at nitriding temperatures.

We have also conceived of a coating in the nature of a paint which may be applied to those portions which are desired to be protected against hardening by nitriding. In such a coating, that is, a paint-like coating in liquid form embodying a metal pigment in a vehicle carrier, the latter comprising a binder together with a flux and solvent for the latter, considerable difficulty is encountered in providing a binder having sufficient bonding properties and in providing a flux particularly suitable from a commercial point of view. This invention is in a broad sense an improvement upon the above method and particularly as to the physical characteristics of the inhibitor. Its general object is to provide an inhibitor to protect those portions of the surfaces of articles which are desired to be left relatively soft while the adjacent unprotected portions are being hardened by the nitriding process.

As previously stated, the nitriding process of hardening involves the use of chemicals at temperatures and under conditions which prevent the use of many substances as inhibitors which might otherwise be desirable. Because of the tendency of the substances to react chemically under nitriding conditions with the metal being treated or with the elements used in the nitriding process in such a manner as to be detrimental to the process or to the metal being treated, these substances are unsuitable. For instance, the temperatures employed in the nitriding proc-

esses tend to cause decomposition of a great many substances which under high temperatures volatilize and are carried out with the exhaust gases. Furthermore, it has been observed that in nitriding furnaces equipped with fans for forced circulation of the ammonia used for nitriding, small amounts of the pigment may be carried along with the fumes formed from the binder or flux probably in the form of a fine dust. This is liable to cause soft spots to occur in the otherwise hardened surface, providing proper precautions are not taken to guard against the carrying off of the pigment and the formation of fumes from the binder and flux.

According to this invention, the parts to be protected, that is remain untreated by the nitriding process, are covered with what might be termed a stop-off or inhibitor or protective coating constituting a covering of a cementitious substance which is not detrimentally affected by the nitriding process, which will withstand the temperatures and conditions, and which will not affect the final suitability of the part being treated. For this purpose it has been found that a cement-like substance of a consistency that permits it being applied readily as with a brush is very desirable and very satisfactory.

However, it is obvious that the mixture may be applied as well by means of a swab, spray, dipping or other suitable means, and after drying, the article may be subjected to the nitriding process. By a cementitious substance is meant a material which due to chemical reaction has the ability to set and harden or form a cement which holds a pigment such as powdered tin in place, the cement being of such a character that it is not subject to decomposition under nitriding conditions.

It has been found that a phosphate cement serves the purpose very satisfactorily. The cement may be formed by mixing a vehicle containing phosphoric acid with a suitable pigment, the pigment being either metal powder or metal powder mixed with non-metallic material. The cement is formed by the reaction of the phosphoric acid on either the metal powder or the non-metallic material or both. The setting and hardening of the cementitious material is of course dependent upon the nature and proportions of the vehicle and pigment and can be governed so as to set slowly and permit the cementitious material being applied conveniently, as a paint. The metal of the protective coating alloys with the steel surface and thus causes a very tight effective bond of the cement to the surface being protected. Inasmuch as the surfaces to be protected are not as a rule sufficiently clean to permit a perfect bonding of the cement with the

surface being treated, it has been found desirable to incorporate a fluxing agent that will serve not only to clean the metal but will provide a better bond between the metal being 5 protected and the cement being applied.

- As a pigment, it has been found satisfactory to use tin or tin together with other metals. Zinc and antimony have been found to give protection also, either alone or with other metals. 10 It is preferable to use a metal or alloy which will not volatilize and sublimate at nitriding conditions and which may be obtained commercially in powdered form. To reduce the amount of metal required it has been found preferable 15 to mix the metal in powdered form with a non-metallic material, for example kieselguhr, silica, kaolin, or similar substances in powdered form. A non-metallic material or filler may be chosen so as to aid in the chemical reaction to form a 20 cement. The ability of the non-metallic material to aid in the formation of a cement is very important in mixtures where the metal powder is not affected by the phosphoric acid solution. The presence of metallic oxides such as zinc 25 oxide, lead oxide, tin oxide or other oxides has proven very effective in the setting or hardening of the cement.

Inasmuch as phosphoric acid reacts very rapidly, it has been found very desirable to employ phosphoric acid salts, for example, ammonium phosphate. The strength of the solution using ammonium phosphate may vary from dilute to very strong concentrations although it has been found that a concentration within the 30 range of 20% to 40% is preferable.

As a flux, any substance or material having the ability to clean and cause the metal of the pigment to unite or closely bond with the surface of the steel alloy being nitrided may be used. 40 Boric acid has been found suitable as it does not volatilize at nitriding temperatures. Zinc chloride may also be used but it is necessary however in this case to keep the vehicle acid in reaction to prevent precipitation of zinc compounds. The use of an acid vehicle also facilitates the application of the inhibitor to the steel. Zinc chloride has also been found to contribute to the cementing properties of the inhibitor. 45 The presence in small amounts of boric acid in a vehicle containing zinc chloride as a flux appears to improve the properties of the cement.

As a specific example, it has been found that a suitable protective coating or inhibitor may be made from the following ingredients within 50 the proportion ranges specified:

|                                | Percent  |
|--------------------------------|----------|
| Ammonium phosphate in solution | 30 to 40 |
| Boric acid in water solution   | 3 to 10  |
| Tin powder                     | 35 to 90 |
| Ground silica                  | 5 to 60  |
| Ground kaolin                  | 1 to 25  |

One example of a satisfactory specific mixture is as follows:

|                                | Percent |
|--------------------------------|---------|
| Ammonium phosphate in solution | 34      |
| Boric acid in water solution   | 8       |
| Tin powder                     | 77      |
| Ground kaolin                  | 3       |
| Ground silica                  | 20      |

Where it is desired to use zinc chloride, the

following ingredients within the proportion ranges have been found satisfactory:

|                                                                                                                               | Percent  |
|-------------------------------------------------------------------------------------------------------------------------------|----------|
| Ammonium phosphate in solution                                                                                                | 20 to 30 |
| Zinc chloride in a sufficiently strong acid solution, preferably hydrochloric acid to dissolve any precipitated zinc compound | 80       |
| Tin powder                                                                                                                    | 35 to 90 |
| Ground silica                                                                                                                 | 5 to 60  |
| Ground kaolin                                                                                                                 | 1 to 25  |

Specific proportions in the following order have been found very satisfactory:

In solution:

|                    | Percent |
|--------------------|---------|
| Ammonium phosphate | 21      |
| Zinc chloride      | 5       |
| Boric acid         | 4       |
| Muriatic acid      | 21      |
| Water              | 49      |

In powder:

|            | Percent |
|------------|---------|
| Tin powder | 70      |
| Kaolin     | 4       |
| Silica     | 26      |

We claim:

1. A protective coating or inhibitor for use in a nitriding process comprising a cementitious material consisting of 30% to 40% ammonium phosphate in solution, 3% to 10% boric acid in water solution, and a pigment including 35% to 90% tin powder, 5% to 60% ground silica and 1% to 25% ground kaolin, the inhibitor deriving its hardening and setting characteristics from the chemical reaction between the liquids and solids. 105

2. A protective coating or inhibitor for use in a nitriding process comprising a cementitious material consisting of substantially 34% ammonium phosphate and 8% boric acid in solution and a pigment of 77% tin powder, 3% ground kaolin and 20% ground silica, the inhibitor deriving its hardening and setting characteristics from the chemical reaction between the liquids and solids. 115

3. A protective coating or inhibitor for use in a nitriding process comprising a cementitious material consisting of 20% to 30% ammonium phosphate and 1% to 7% zinc chloride in acid solution and a pigment of 35% to 90% tin powder, 5% to 60% ground silica and 1% to 25% ground kaolin, the inhibitor deriving its hardening and setting characteristics from the chemical reaction between the liquids and solids. 125

4. A protective coating or inhibitor for use in a nitriding process comprising a cementitious material consisting of 20% to 30% ammonium phosphate and 1% to 7% zinc chloride in hydrochloric acid and a pigment of 35% to 90% tin powder, 5% to 60% ground silica and 1% to 25% ground kaolin, the inhibitor deriving its hardening and setting characteristics from the chemical reaction between the liquids and solids. 135

5. A protective coating or inhibitor for use in a nitriding process comprising a cementitious material consisting of a liquid of substantially 21% ammonium phosphate, 5% zinc chloride, 4% boric acid, 21% hydrochloric acid and 49% water, and a pigment of 70% tin powder, 4% ground kaolin and 26% ground silica. 140

HAROLD A. ECKMAN.  
HENRY W. MAACK.